

1

3,345,207

**NON-WOVEN FABRIC PREPARED WITH METHYLOL AMIDES OF AN ADDUCT FORMED BETWEEN A MALEYL COMPOUND AND AN ETHYLENICALLY UNSATURATED ALIPHATIC COMPOUND**

George W. Cogswell and Lester P. Hayes, Decatur, Ill., assignors to A. E. Staley Manufacturing Company, Decatur, Ill., a corporation of Delaware  
No Drawing. Filed June 20, 1963, Ser. No. 289,384  
18 Claims. (Cl. 117—140)

This invention relates to bonded non-woven fibrous or filamentous products having a carded fiber structure or comprising fibrous mats in which the fiber or filaments are distributed haphazardly or in random array. The invention also relates to methods for producing the bonded non-woven fibrous products or shaped articles therefrom. The bonded non-woven fibrous products are useful in the production of articles of either flat or three-dimensional shape, including insulating material and the like as will be described more particularly hereinafter.

Hereinafter, the expression "random array" is intended to include the array of fibers in a carded web wherein partial orientation is frequently present as well as other arrays in which the fibers are in a completely haphazard distributional relationship.

Heretofore, binders of natural rubber latex and aqueous dispersions of synthetic rubbers, such as butadiene copolymerized with styrene, acrylonitrile and so on have been suggested as binders for bonding the fibers in non-woven fabric structures; but these materials have various disadvantages. These rubbery binders produce a rubbery hand which appears to be the result of a complete suppression of the fibrous character insofar as the feel of the product is concerned. When binders of polyvinyl acetates, chlorides, or their copolymers are used, the hand becomes papery, by which is meant that the product has a noisy, crisp, brittle hand and conveys the impression of thinness and fragility. Further, the water-resistance and solvent resistance of some of these products leaves something to be desired. The application of thermoplastic polymers of monomers such as simple esters of acrylic or methacrylic acid produces products in which the binder remains permanently thermoplastic with consequent tendency to change when subjected to excessive temperatures. The simple polymers of acrylic and methacrylic acid esters are also characterized by relatively poor adhesion to hydrophobic types of fibers, such as nylon, vinyl resin fibers, cellulose esters, and polyesters such as polyethylene glycol terephthalate. Furthermore, many of the binders heretofore employed, including the aqueous dispersion of rubber, synthetic rubbers and acrylic ester polymers, have a strong tendency to migrate to the surface of the fibrous products during drying of the products to which the dispersion have been applied. In addition to the foregoing, many of these binders, particularly aqueous dispersions of the polyacrylic esters, are relatively expensive.

The object of this invention is to provide fibrous products made with an inexpensive binder which can be applied by way of an aqueous system within the disadvantages mentioned above that are characteristic of previously applied aqueous binder systems. Another object of this invention is to provide a bonded fibrous product of non-woven character in which the binder is adapted to be converted to an infusible and insoluble condition as by heating with or without the presence of a suitable catalyst as will be pointed out more particularly hereinafter. A further object of this invention is to provide bonded fibrous products of non-woven character wherein the binder may be substantially uniformly distributed through the body of the structure and has reduced tendency to migrate to the surfaces of the structure.

2

A still further object of this invention is to provide a low cost auxiliary binder for use with conventional non-woven binders, which increases the water and solvent resistance of binders such as polyvinyl acetate, which increases the adhesion of binders such as the simple acrylate polymers, which prevents the flow of thermoplastic binders, etc.

According to the present invention, it has been found that aqueous dispersions of the reaction product of formaldehyde with amide adducts of alpha, beta-ethylenically unsaturated dicarboxy compounds (maleyl compounds) and ethylenically unsaturated compound having a chain of at least 10 carbon atoms are capable of bonding fibers of a non-woven fibrous product. As explained in detail in commonly assigned application Ser. No. 264,069, filed Mar. 11, 1963, these methyol amide adducts can be prepared by (1) forming an adduct of an alpha,beta-ethylenically unsaturated dicarboxy compound (maleyl compound) and a long chain ethylenically unsaturated compound having a chain of from 10—24 carbon atoms; (2) reacting said adduct with a basic nitrogen compound, which contains at least two active hydrogen atoms bonded to the same or different nitrogen atoms in the same molecule, and (3) reacting the product of step (2) with a formaldehyde source.

In the description that follows, the words "dispersing" and "dispersion" are used in a generic sense to be inclusive of the words "suspending," "dissolving," "suspension," and "solution." The words "ammonia" and "ammonium hydroxide" are used interchangeably. The term "formaldehyde" is used in a generic sense to be inclusive of monomeric formaldehyde and formaldehyde-generating materials. The term "potentially reactive carboxy group" includes the following reactive groups: the amide group, the methyol amide group, the anhydride group, the free carboxylic acid group and carboxylic acid salt groups.

The long chain ethylenically unsaturated compounds can be substituted or contain various other groups such as carboxyl groups, carboxylate groups, halo groups, acyloxy groups, alkoxy groups, aryloxy groups, tertiary amino groups, quaternary ammonium groups, etc. The preferred long-chain ethylenically unsaturated compounds of this invention are the readily available, naturally occurring polyunsaturated glyceride oils (which are considered as having carboxylate groups) having from 10 to 24 carbon atoms in the unsaturated long chain, such as soybean oil, corn oil, cottonseed oil, hempseed oil, tung oil, safflower oil, peanut oil, linseed oil, tobacco seed oil, cod oil, herring (or menhaden) oil, dehydrated castor oil, etc. The glyceride oils and the esters of other unsaturated long chain acids, such as the linoleic acid esters of trimethylol propane and tall oil fatty acid esters of pentaerythritol, are preferred since they contain a relatively large number of ethylenic double bonds available as sites for adduct formation. In general, those compounds having on an average at least two and preferably three to nine non-conjugated ethylenically unsaturated groups per molecule are preferred. These can be thought of as being esters of a polyhydric alcohol (e.g. ethylene glycol, trimethylol ethane, sorbitol, inositol, etc.) having from 2 to 6 hydroxyl groups with ethylenically unsaturated fatty acid chains of from 10 to 25 carbon atoms.

Other useful long chain fatty compounds include methyl oleate, 2-ethyl hexyl ester of tall oil fatty acids, oleic acid, linoleic acid, linolenic acid, ammonium linoleate, N-unsubstituted linoleamide, octadecene-9, 1-chlorodecene-4, 1-bromoocadecene-9, 1-chlorotetraocadecene-9, 1-nitroocadecene-9; N,N-dimethyllinoleamide, N,N-linoleimide, N,N-linolenimide, N,N-dimethyl-N,N-dilinoleylamine, N-methyl-N,N-dilinoleylamine, 10-carboxydecene-2, 1-acetoxyocadecene-4, 1-phenoxyocadecene-9, 1-propoxyocadecene-9, etc.

The maleyl compound (alpha, beta-ethylenically unsaturated dicarboxy compound) can be maleic anhydride, maleic acid, fumaric acid, dimethyl maleate, monomethyl hydrogen maleate, mono-2-ethylhexyl hydrogen maleate, citraconic acid citraconic anhydride, itaconic acid itaconic anhydride, ethyl maleic acid, maleimide, maleamic acid, etc. Of these, maleic anhydride is preferred because of (1) its low cost, (2) the ease with which it forms adducts in almost quantitative yields, and (3) the high concentration of amide groups which result from the reaction of the anhydride adduct with a basic nitrogen compound. While maleic acid, which forms the anhydride, under the conditions of adduct formation has most of the advantages of maleic anhydride, it is twice as expensive as the anhydride. Fumaric acid, which approaches the cost of maleic anhydride on a weight basis, requires considerably more severe reaction conditions to form an adduct and, even then, the yield is lower. Further, adducts prepared from free dicarboxylic acids that are not capable of forming an anhydride under the conditions of the maleation reaction and from half-esters and diesters produce amides with a lower concentration of amide groups after treatment with a suitable basic nitrogen compound than corresponding adducts containing the same concentration of carboxy groups in the anhydride form. It goes without saying that diesters are only suitable in this invention when at least some of the carboxy groups in the diester adduct are saponified during or before the addition of the basic nitrogen compound to permit amide formation. Citric acid and malic acid which form alpha-, beta-ethylenically unsaturated dicarboxy compounds under the conditions of the maleation reaction can also be used in this invention.

Ammonia, which can be employed as gaseous ammonia or in the aqueous ammonium hydroxide form, is the preferred basic nitrogen compound because of its low cost, availability, high vapor pressure in water, the ease with which it forms amides and the ease with which its amides form methylol groups. Various primary amines; such as methyl amine, ethyl amine, and butyl amine; primary and secondary polyamines; such as ethylene diamine, diethylene triamine, propylene diamine and N,N'-dimethyl-ethylene diamine; can be used to partially or completely replace ammonia. All of these amines contain at least two active hydrogen atoms which may be bonded to the same or to different nitrogen atoms in the same molecule.

Formaldehyde, generally as formalin, is the preferred source of formaldehyde. Polymeric forms of formaldehyde, such as trioxane and paraformaldehyde, are decidedly inferior to formaldehyde. These polymeric groups must be employed at much higher temperatures than the

monomeric formaldehyde. Of course, the polymeric form is equivalent to the monomeric form if it is first converted to the monomeric form before addition to the amide adducts. Reaction products of formaldehyde with basic nitrogen compounds of the preceding paragraph (e.g. hexamethylenetetramine) are decidedly poorer than the individual reactants. Even in those cases where ammonia has been employed to form the amide prior to the addition of hexamethylenetetramine, higher temperature must be employed to form the desired methylol amide than when monomeric formaldehyde is used. Further, the detergent resistance of non-woven fabrics prepared with formaldehyde condensation products are inferior to the detergent resistance of non-woven fabrics prepared from monomeric formaldehyde.

In somewhat greater detail the adduct is formed by reacting the long chain ethylenically unsaturated fatty compound and the maleyl compound at a temperature of about 150° C. to 300° C. in an open vessel or under pressure in an autoclave. While maleic anhydride forms an adduct in almost quantitative yields in an open vessel, other maleyl compounds, such as dibutyl maleate, give considerably better yields when the reaction is carried out under pressure.

The ratio of maleyl compound to ethylenically unsaturated long chain fatty compound in the reaction vessel can range from about 0.1 to 2 moles or more of maleyl compound per equivalent of unsaturation in the long chain fatty compound, depending upon the choice of reactants and the desired properties of the products. For example, the preferred naturally occurring glyceride oils, such as soybean oil or linseed oil, can be reacted with from about 10% to 45% by weight of maleic anhydride to form adducts containing from about 1.0 to 4.5 maleic anhydride moieties per molecule of glyceride oil. (The resulting maleic anhydride portion of the glyceride oil adduct comprises from about 10% to 3% by weight of the product.) The properties of the various members vary, as follows, depending upon the level of maleation.

Maleated glyceride oils, which contain about 10% by weight maleic anhydride or about 1.0 mole of anhydride per mole of glyceride oil, form stable suspensions in aqueous ammonium hydroxide while those containing in excess of about 14% by weight maleic anhydride or about 1.5 moles of anhydride per mole of glyceride oil are soluble in aqueous ammonium hydroxide. Methylol amides at the same level of maleation have essentially the same dispersibility characteristics in aqueous base as the anhydride adduct from which the methylol amide is formed. Other things being equal, non-woven fabrics prepared with glyceride oil methylol amides vary as the level of maleation increases as follows:

TABLE I

| Average total number of potentially reactive carboxy groups per molecule of glyceride oil | Maleate moieties per molecule of glyceride oil | Weight percent of maleic anhydride in the methylol amide precursor | Properties of non-woven fabric                                      |
|-------------------------------------------------------------------------------------------|------------------------------------------------|--------------------------------------------------------------------|---------------------------------------------------------------------|
| 2                                                                                         | 1.0                                            | 10                                                                 | Tacky material without strength.                                    |
| 3                                                                                         | 1.5                                            | 14                                                                 | Soft, oily, water-resistant fabric with low strength.               |
| 3.7                                                                                       | 1.85                                           | 17                                                                 | Soft, oily, water-resistant fabric with fair strength.              |
| 5                                                                                         | 2.5                                            | 22                                                                 | Water-resistant fabric having good strength and solvent resistance. |
| 6                                                                                         | 3                                              | 24.5                                                               | Flexible, water-resistant, solvent-resistant fabric.                |
| 8.7                                                                                       | 4.85                                           | 33                                                                 | Do.                                                                 |

In general, the methylol amides based upon unsaturated long chain carboxylic acid esters of polyhydric alcohols containing a total of from about 2 to 4 potentially reactive carboxy groups (carboxylate salts, amide and methylol amide groups) per molecule (preferably about 3.5 to 4) are suited particularly for use as non-woven binders for disposable wiping cloths (industrial dust-catching cloths). These cloths are not laundered because of their low cost, poor detergent resistance and soft absorbent character. For the most part, laundering costs more than the cloths themselves.

The methylol amides based upon unsaturated fatty acid esters of polyhydric alcohols containing a total of about 4 to 9 potentially reactive carboxy groups per molecule (preferably about 5 to 7) are suited for use as the vehicle for non-woven binders having excellent solvent-resistance and detergent resistance and these are the preferred products of this invention.

The maleated long chain fatty material can be converted to the amide by a variety of techniques. For example, an anhydride adduct, such as that resulting from the maleation of a naturally occurring glyceride oil and maleic anhydride or maleic acid, can be converted to the amide form in any of the following ways: (1) stirring the anhydride adduct in an atmosphere of ammonia until the exothermic reaction ceases, (2) adding concentrated ammonium hydroxide (28% aqueous solution, for example), to the anhydride adduct and stirring until the adduct disperses, (3) adding the anhydride adduct to concentrated ammonium hydroxide and stirring until the adduct disperses, (4) mixing the anhydride adduct with a calculated amount of water and then bubbling a sufficient amount of ammonia gas into the system to disperse the anhydride adduct, (5) mixing the anhydride adduct with a calculated amount of water, opening the anhydride ring by heating and then adding ammonia gas or aqueous ammonium hydroxide to disperse the adduct.

It has been found that adding the anhydride adduct to concentrated ammonium hydroxide yields the highest concentration of amide groups. For example, when the above illustrative anhydride adduct (glyceride oil and maleic anhydride) is added to a concentrated aqueous ammonium hydroxide solution containing two molecules of ammonium hydroxide per anhydride group in the adduct, about 85% of the anhydride groups (42.5% of the carboxy groups) are converted to monoamide groups. The remainder of the ammonium hydroxide is present as the ammonium salt. On the other hand, when the ammonium hydroxide is added to the adduct in the same proportion, about 60% of the anhydride groups (30% of the potentially reactive carboxy groups) are converted to monoamide groups. About 30% of the anhydride groups are converted to monoamide groups when concentrated ammonium hydroxide is added to the anhydride adduct in a ratio of one molecule of ammonium hydroxide per anhydride group.

Still lower yields of amide are obtained if the anhydride ring is opened prior to the addition of ammonium hydroxide. For example, when the anhydride ring of the same adduct is first broken by heating with water, the addition of ammonium hydroxide to the adduct (in a ratio of one molecule of ammonium hydroxide per anhydride ring produces only 15% of amide-containing anhydride groups (7.5% of the carboxy groups).

While the combined number of potentially reactive carboxy groups per molecule of fatty material has a pronounced effect on the properties of the final non-woven fabric, the ratio of amide groups to carboxylate salt groups has a smaller effect. For example, non-woven fabric based upon glyceride oil adducts having on an average 0.9 amide group and 5.1 carboxylate salt groups per molecule have properties quite similar to non-woven fabrics based upon glyceride oil adducts having on an average from about 1.8 to about 2.6 amide groups and correspondingly 4.2 to 3.4 carboxylate salt groups (6

potentially reactive carboxy groups per molecule). Other things being equal, the latter products have somewhat better detergent resistance, solvent resistance, and higher tensile strength. Accordingly, products having higher ratios of amide groups to carboxylate salt groups are preferred.

The amide adduct, which has preferably been dispersed in water, is then reacted with formaldehyde or a compound capable of generating formaldehyde preferably by adding the formaldehyde source (usually formalin or paraformaldehyde depolymerized to the monomeric form) to the amide adduct or by adding the amide adduct to the formaldehyde source. This reaction can be carried out in a sealed vessel at moderate temperature (5° C. to 75° C.) or in an open vessel. A sufficient concentration of formaldehyde is added in this step to provide at least 0.7 mole of formaldehyde per each equivalent of nitrogen containing compound bearing a nitrogen atom bonded directly to hydrogen (each NH group) in the aqueous composition.

Excellent results have been obtained by adding at least about 0.8 mole of formaldehyde for each mole of basic nitrogen containing compound, which contains two hydrogen atoms bonded directly to nitrogen, used to form the amide. In this way essentially all the ammonium ions, etc. in the reaction medium are converted to non-volatile nitrogen and the methylol amide adduct is precipitated from the aqueous reaction medium as a water-insoluble hydrate. This frequently has a dough-like consistency. The formation of this precipitate is visual evidence that a sufficient concentration of formaldehyde has been added to the amide adduct.

If less than 0.7 mole of formaldehyde per each equivalent of nitrogen-containing compound is added to the aqueous amide adduct, the methylol amide-bound non-woven fabric does not have water resistance and detergent resistance. In fact, the water resistance and detergent resistance is in some cases only slightly better than that if the non-woven fabric had been prepared with an amide adduct, which had not been reacted with formaldehyde.

After the formaldehyde reaction, the resultant methylol amide adduct is neutralized or made basic by the addition of a suitable basic material, preferably ammonium hydroxide or a volatile amine. Any precipitated methylol amide is thereby redispersed.

Non-volatile alkali is not preferred since non-woven fabrics based thereon have poorer water resistance and detergent resistance. Diamines, such as ethylene diamine, are advantageously employed with ammonia in order to give the cured products a somewhat softer, more flexible character. Ethylene diamine is particularly advantageous since it acts as a wetting agent for viscose webs. Ethylene diamine is preferably used in a concentration of from about .05 to .25 mole per each mole of maleyl compound in said methylol amide.

The methylol amide binders of this invention can be used in dispersions containing from about 1% to 60% by weight binder solids. It is generally preferred, however, that the binder solids be in the range of about 5% to 30% by weight in order to facilitate the application of the binder to the fibers by spraying, dipping, or by transfer rolls.

The binders of the present invention are characterized not only by good adhesion to hydrophilic fibers like cotton, regenerated cellulose rayons and the like, but they are also characterized by excellent adhesion to hydrophobic types of fibers, such as the nylons, especially poly(hexamethylene adipamide), the vinyl resins such as copolymers of vinyl chloride with vinyl acetate or with acrylonitrile, polymers of 70 to 90% acrylonitrile with other monomers such as vinyl chloride, vinyl acetate, any of the vinyl pyridines such as 2-vinyl pyridine or mixtures of such auxiliary comonomers, polyesters, such as poly(ethylene terephthalate), and cellulose esters such as cellulose acetate, cellulose acetate propionate, cellulose

acetate butyrate and so on. Because of the characteristic adhesion of the binder of the present invention to both hydrophilic and hydrophobic types of fibers, the fibrous products are characterized by excellent resistance to "pilling" and abrasion. The binder of the present invention is adapted to be dried and then cured to insoluble and infusible condition so that the bonds cannot be disturbed even under severe conditions of heat. While the binder may be preferentially applied, if desired, to portions of the fibrous product, such as one or both of the faces thereof, it is characteristic of the binder of the present invention that if such preferential treatment is not desired, substantially uniform distribution may be obtained because of the reduced tendency of the binder after initial distribution throughout the body of the fibrous product to migrate to the surfaces thereof during drying.

The binder of the present invention may also contain: dyes of water-dispersible type if coloration is desired; lubricants and/or softeners of water-dispersible type. Emulsified polyethylene is the preferred softener for use with the methylol amides of this invention. The emulsified polyethylene can comprise from about 1 to about 100 parts on a dry solids basis (D.S.B.) for each 100 parts of methylol amide (D.S.B.). Best results have been obtained using from 30 to 60 parts (D.S.B.) for each 100 parts methylolamide (D.S.B.).

The cured or insolubilized binders of this invention, wherein said binder has on an average at least 4 potentially reactive carboxy groups per molecule (preferably at least 5) are unaffected by water or organic solvents, such as perchloroethylene and carbon tetrachloride, even at molding temperatures, whereby the bonded fibrous products are adapted to be used as molding preforms or molding inserts for the production of molded articles from various thermosetting resins as will be pointed out in more detail hereinafter. After cure the binders are also free of cold flow and are resistant to flow at elevated temperatures, whereby shifting of the fibers or filaments in the bonded products is almost completely prevented even at elevated temperatures during subsequent molding when such products are used as reinforcing inserts or preforms.

In accordance with the present invention, the fibers of the non-woven web may comprise wool or may consist entirely of non-proteinaceous fibers which are incapable of felting. The fibers are present in the form of a so-called "non-woven" mat in which they are haphazardly distributed, or the mat may be formed by carding when the fibers are of such a character, by virtue of length and flexibility, as to be amenable to the carding operation. Natural fibers like wool, linen, silk, jute, sisal, ramie, hemp, and cotton may be used, as well as many artificial fibers or filaments including rayon, those of cellulose esters such as cellulose acetate, vinyl resin fibers such as those of polyvinyl chloride, copolymers of vinyl chloride with vinyl acetate, vinylidene chloride or acrylonitrile containing a major proportion of vinyl chloride in the polymer molecule, polyacrylonitrile and copolymers of acrylonitrile with vinyl chloride, vinyl acetate, methacrylonitrile, vinyl pyridine, or with mixtures of such comonomers and containing a major portion from 75 to 95% of acrylonitrile in the copolymer molecule; also condensation polymers such as polyamides of nylon type, polyesters such as ethylene glycol terephthalate polymers and the like. The thin web or fleece obtained from a single card may be treated in accordance with the present invention, but generally it is necessary and desirable to superpose a plurality of such webs to build up the mat to sufficient thickness for the end use intended particularly in the making of heat insulation. In building up such a mat, alternate layers of carded webs may be disposed with their fiber orientation directions disposed at 60° or 90° angles with respect to intervening layers.

Mats may also be formed by the deposition of fibers, either natural or artificial, from an air stream. Thus, con-

tinuous filaments may be fed to a cutter or breaker which discharges the fibers into the discharge side of a blower. Suitable conduits are provided to guide the fibers to a collecting screen or air-pervious structure for collecting the fibers in the form desired. The screen may be in the form of an endless traveling belt passing through the lower portion of a tower into the upper portion of which the blown fibers are introduced by the conduit work. A suction box may be disposed beneath the upper course of the traveling screen to assist in the disposition of the fibers thereon. Instead of having a traveling flat screen, a stationary formed screen may be used. For example, it may take the form of a hat-shaped cone such as that used in the felt hat-making industry. Alternatively, it may have any other form suitable to produce the desired shape of the fibrous product, such as a rectangular tray. Again, suction may be applied beneath the screen to assist deposition of the fibers thereon.

The fibers and filaments may be formed by direct spraying from a solution or molten mass thereof. This is a conventional procedure for the formation of glass fibers or mineral wool fibers as well as those of nylon or of thermoplastic materials, such as vinyl resins of the type mentioned hereinabove, adapted to be dissolved in a suitable solvent, such as acetone or dimethyl formamide, or to be melted. The solution or melt is, of course, directed to suitable nozzles or jet-forming orifices and a high pressure fluid stream, such as of cold or hot air or of inert gases such as nitrogen or even of steam, is directed against the stream or streams of filament-forming material to disrupt them and coagulate them as fibers in the vicinity of the orifices. Electrostatic spinning methods may also be employed for this purpose. As in the case of the use of blowers, the disrupted and dispersed fibers may be directed to the top of a settling tower and be allowed to settle with the aid of suction devices upon a suitable traveling or stationary screen at the bottom of the tower. This procedure is adaptable to the production of fibers of siliceous materials such as glass or mineral wool as well as to thermoplastic resin fibers mentioned above.

Another procedure may involve the extrusion of continuous filaments either from solutions of the filament-forming material or from molten masses thereof, and the cutting or breaking of the filaments to fibers of a predetermined length which may be fed to a hopper at the top of a settling tower into which they may be discharged by conventional feeding devices, and at the bottom of which a traveling or stationary screen may be located for collection of the fibers.

The fibers and filaments that may be used in the present invention may be natural or artificial as stated above. The selection of the particular material of which the fiber is made frequently depends upon the intended use of the product. For example, siliceous fibers are extremely valuable in the production of molded articles because of the exceptional strength obtained by their use. However, when the bonded fibrous products are used for filtration purposes, fibers of certain resins may be preferred to provide resistance to attack by acids or alkalies that may be present in the liquids to be filtered. Thus, polymers containing a high percentage of acrylonitrile or of vinyl chloride or even of such highly halogenated resins as polytetrafluoroethylene or poly(chlorotrifluoroethylene) may be more useful in such cases. For certain purposes, it may be desirable to form the fibrous products from a mixture of fibers of different types. An example is the use of a mixture of thermoplastic fibers of potentially adhesive character with other fibers which lack such potentially adhesive character. A fibrous product comprising such a mixture may be heated to the appropriate temperature to render the potentially adhesive fibers tacky to effect binding of the fibers in the product by this procedure as well as by the binders of the present invention.

The binder dispersion may be applied to the dry fibers after the formation or deposition of the web or mat so

as to penetrate partially into or completely through the interior of the fibrous products. Alternatively, the binder dispersion may be applied to the fibers as they fall through a settling chamber to their point of deposition. This result is advantageously obtained by spraying the binder dispersion into the settling chamber at some intermediate point between the top and the bottom thereof. By so spraying the fibers as they descend to the point of collection, it is possible to effect a thorough distribution of the binder among the fibers before they are collected into the product. In the production of certain fibrous products wherein a hot molten mass of a polymer, such as nylon or a fused siliceous mass or glass, is disrupted by jets of heated air or steam, the binder dispersion may be sprayed directly on the fibers while still hot and very shortly before their deposition so that quickly after deposition the binder is set and bonds the fibers in proper relationship. Preferably, however, application of the binder dispersion to the fibrous product is made at room temperature to facilitate cleaning of the apparatus associated with the application of the binder dispersion. The binder dispersion may be applied to one or both surfaces of the fibrous product or it may be distributed through the interior as well. If desired, the binder of this invention can be applied as a size to the fibers, prior to the formation of the web.

The binder of the present invention may be used in conjunction with other binders. For example, the methylol amides of this invention can be used in conjunction with homopolymers and copolymers of vinyl acetate, vinyl chloride, vinylidene chloride, acrylonitrile, styrene, acrylic and methacrylic acid esters; e.g. the methyl, ethyl, propyl or butyl esters thereof, and so on. The methylol amide of this invention may comprise from 1 to 100% of the binder solids. Compositions comprising from about 5% to 50% methylol amide and from about 95% to 50% polyvinylacetate, give rise to non-wovens having markedly better water-resistance and solvent resistance than non-wovens based solely on polyvinyl acetate. Likewise, the adhesion of acrylate binders is improved by small amounts of methylol amide.

The fibrous product of non-woven character may contain from about 1/2 to about 200% by weight binder on the weight of the fibers depending on the purpose for which the product is to be used. When the binder is to serve mainly to bond the fibers together to form a coherent unitary structure in which the maximum porosity is retained together with a minimum change of natural fiber hand, there may be employed from 1/2 to 1% by weight of binder solids on the fiber, the lower proportion, of course, giving the maximum porosity possible and providing a minimum change in the natural fiber hand although even with the larger proportion in this range, the porosity is mainly retained and the fiber hand is still evident. It is characteristic of the binder applied in the proportions just stated that there is relatively little or no "window paning," that is, the interstices between fibers are left open leaving a highly porous bulky product. "Window paning" does not result since the methylol amides employed in this invention are actually dissolved in the aqueous medium, unlike prior emulsion binders. Of course, the density of the product can be effected or modified by the application of pressure prior to or, in many cases, even after the curing of the product.

Fibrous products of non-woven character using from 2 to 30% by weight of the binder of the present invention on the weight of the fiber are generally quite useful in garments, for example as interlining fabrics for coats, dresses, and so on, or to provide outer wearing apparel fabrics, such as blouses, skirts, shirts, etc. The garments made of these fabrics need little or no ironing, or pressing, to restore their appearance, shape and hand after hand-washing, machine-laundering and drying operations. Besides the apparel uses mentioned above, fibrous products of the invention in which 1/2 to 20% by weight of

binder on the weight of fiber is employed, find many light industrial uses as wiping cloths, lining materials for packaging as filters, and packings and gaskets for industrial machinery.

5 Fibrous products of the present invention, in which 20 to 150% by weight of the binder on the weight of fiber is used, are especially useful for heavy industrial uses where durability and resistance to wear are desired, such as in industrial gaskets, packings, filters, and so on. The products containing 20 to 75% of the binder of the present invention on the weight of the fiber are useful as laminating layers, either as interlayers or backing sheets in conjunction with plastic films and sheets as of polyethylene, nylon, and so on, or in conjunction with textile fabrics of woven, braided, knitted, or felted character.

10 To render the binder infusible, curing temperatures in the range of about 110° C. to 350° C. may be used. Generally, temperatures in the range of 120° to 200° C. for about 1 to 10 minutes are sufficient.

15 Catalysts, such as melamine dissolved in formalin, hexamethylene tetramine, ammonium p-toluene sulfonate, zinc ammonium acetate, zinc fluoroborate, zirconium ammonium acetate, ammonium vanadate, ammonium molybdate, etc. can be used to speed up the cure. The catalyst can be used in a concentration up to 5% by weight based on the dry weight of the methylol amide in order to speed up the cure or permit the use of lower cure temperatures. In the absence of a catalyst the rate of cure is impractically slow at temperatures much below 140° C.

20 The following examples are merely illustrative and should not be construed as limiting the scope of the invention.

#### Example I

25 A 10" by 20" piece of 100 percent viscose carded web weighing about 0.3 ounce per square yard was sandwiched between supporting glass-fiber screening and then impregnated by dipping the sandwich into a 15 percent active material solution of a methanol amide (prepared from soybean oil, maleic anhydride, ammonia and formaldehyde, as described before) having on an average 6 potentially reactive carboxyl groups per molecule. The impregnated sandwich was then passed through the steel and hard rubber rolls of a two-roll Birch padder at 25 p.s.i. roll pressure. The supporting glass fiber screening was removed and the impregnated web was placed on paper and dried at 40° C. for one hour. After drying, the web was cured at 150° C. for four minutes. The web was then 30 calendered twice on the padder at 65 p.s.i. with the steel rolls immersed in hot water 140° F. and dried for one hour at 40° C. The resulting non-woven fabric, which was about 60 parts by weight fiber and 40 parts by weight binder, had a texture similar to a non-woven web prepared with polyvinyl acetate. However, the web had markedly better organic-solvent resistance, detergent resistance and water resistance than a non-woven web prepared with polyvinyl acetate. Further, the non-woven fabric did not have the objectionable noisy hand characteristic of non-woven fabrics prepared with polyvinyl acetate binders.

35 40 45 50 55 60 The methylol amide used in this example was prepared in the following manner.

65 Eight hundred and eighty-four grams of bleached soybean oil (1 mole) was heated to 230° C. in a three-necked flask equipped with a stirrer, reflux condenser and addition port. After 294 grams (3 moles) of liquid maleic anhydride was added through the addition port over a period of one and one-half hours, the composition was heated to 250° C. and held there for 15 minutes. The maleated oil, after cooling to about 50° C. was 70 75 added to 700 grams of aqueous ammonium hydroxide (6 moles ammonia) and then the reactants were maintained at between 25-50° C., thereby dissolving the maleated oil. It was determined, by distilling off ammonia from a slightly basic sample of the solution, that about 42.5%

of the potentially reactive carboxy groups (85% of the starting anhydride groups) had been converted to the amide form. Five hundred and fifteen grams of formalin (6.3 moles formaldehyde) were added rapidly to the solution and the pH of the aqueous system dropped to about 5 to 5.5 precipitating the methylol amide as a water-insoluble hydrate. The water-insoluble hydrate was redissolved by slowly adding 143 grams of aqueous ammonium hydroxide (2.1 moles ammonia) while maintaining the exothermic reaction at about 50° C. The solution had a pH of about 7. Then 21.2 grams ethylene diamine (0.35 mole) and 52.0 grams aqueous ammonium hydroxide (0.77 mole ammonia) were added to adjust the pH of the aqueous solution of methylol amide to a pH of 7.5-8.5. The final product was approximately 60% active material.

*Example II*

(A) Example I was repeated with essentially the same results except that the impregnated web was dried at 110° C. for 5 minutes and cured at 150° C. for 2 minutes instead of being dried at 40° C. for 1 hour and cured at 150° C. for 4 minutes.

(B) When Example I was repeated using a roll pressure of 5 p.s.i. on the Birch padder the resulting non-woven was approximately 25 parts by weight fiber and 75 parts by weight binder.

(C) When Example I was repeated using a roll pressure of 60 p.s.i. on the Birch padder the resulting non-woven was approximately 90 parts by weight fiber and 10 parts by weight binder.

*Example III*

A non-woven disposable dust cloth was prepared by the method of Example I using a methylol amide having on an average 3 potentially reactive carboxyl groups per molecule. The methylol amide was prepared by the method of Example I by reacting, in this order, 884 grams of bleached soybean oil (1 mole), 150 grams maleic anhydride (1.53 moles), 258.5 grams water, 177.8 grams aqueous ammonium hydroxide (2.6 moles ammonia), 452.9 grams formalin (5.6 moles formaldehyde), 204 grams aqueous ammonium hydroxide (3 moles ammonia), 18.6 grams ethylene diamine (0.3 mole) and 45.5 grams aqueous ammonium hydroxide (0.7 mole ammonia).

The disposable wiping cloth was composed of about 55 parts by weight fiber and 45 parts by weight binder. It had a soft oily hand and was resistant to water and carbon tetrachloride.

*Example IV*

Example III was repeated except that no ethylene diamine was used in the preparation of the methylol amide. The disposable wiping cloth, which was composed of about 88 parts by weight fiber and 12 parts binder, had less strength and solvent resistance. This example illustrates that the incorporation of ethylene diamine in the methylol amide results in better wetting of viscose web.

*Example V*

Example I was repeated except that one-third of the methylol amide in the impregnating bath was replaced by 5 parts, dry solids basis, emulsified polyethylene. The non-woven fabric had essentially the same properties as the non-woven fabric prepared in Example I except that the non-woven fabric of this example had a soft hand. This non-woven fabric had all the properties of a non-woven fabric prepared with the most expensive acrylate polymers.

Essentially the same results were obtained when the viscose webs was replaced by a 100 percent Acrlan (polymerized acrylonitrile) web, an 80% acetate-20% nylon blend and a 100% polyethylene terephthalate web.

*Example VI*

25 Example I was repeated using an impregnating bath containing 1.8% (active ingredients) methylol amide of Example I and 13.2% (dry solids basis) polyvinyl acetate emulsion. The non-woven fabric had markedly better organic-solvent resistance (carbon tetrachloride), detergent 30 resistance and water resistance than a non-woven fabric prepared with 15% (dry solids basis) polyvinyl acetate. Further, the non-woven fabric was not noisy.

*Example VII*

35 This example illustrates the compatibility of the methylol amide of Example I with a number of commercially available polymers, which compositions can be used to prepare suitable non-woven fabrics. The methylol amide of Example I (60% active material) and the various  
40 commercially available polymers were compounded on an "as is" basis and at 20% total solids. The compatibility of the various systems is set forth below in Table IX. In the table, the top line, or "A" line, represents the "as is" composition; the bottom line, or "B" line, represents the  
45 composition at 20% total solids. "I" stands for incompatible; "PC" stands for partly compatible; "C" stands for compatible; "T.S." for total solids and "\*" stands for high viscosity.

TABLE IX

| Test Polymer                    | Ratio of Methylol Amide of Example I to Polymer |                        |                        |                     |                        |                        |                     |                        |                        |                     |
|---------------------------------|-------------------------------------------------|------------------------|------------------------|---------------------|------------------------|------------------------|---------------------|------------------------|------------------------|---------------------|
|                                 | 1:4                                             |                        |                        | 1:1                 |                        |                        | 4:1                 |                        |                        |                     |
|                                 | Imme-<br>di-<br>ate                             | 8 hours on<br>standing | 24 hours<br>at 125° F. | Imme-<br>di-<br>ate | 8 hours on<br>standing | 24 hours<br>at 125° F. | Imme-<br>di-<br>ate | 8 hours on<br>standing | 24 hours<br>at 125° F. | Imme-<br>di-<br>ate |
| Darex 81L (55.8% T.S.)          | A                                               | I                      | I                      | I                   | C                      | PC                     | PC                  | C                      | PC                     | PC                  |
| Polyvinyl Acetate               | B                                               | C                      | I                      | PC                  | C                      | PC                     | I                   | C                      | I                      | PC                  |
| Elvacet 81-900 (55% T.S.)       | A                                               | C                      | I                      | C                   | C                      | PC                     | C                   | CC                     | PC                     | PC                  |
| Polyvinyl Acetate               | B                                               | C                      | C                      | I                   | PC                     | PC                     | I                   | CC                     | I                      | I                   |
| Polyco-694 (56% T.S.)           | A                                               | CC                     | I                      | I                   | CC                     | I                      | I                   | CC                     | I                      | I                   |
| Polyvinyl Acetate               | B                                               | CC                     | C                      | PC                  | CC                     | CC                     | PC                  | CC                     | PC                     | PC                  |
| Pliolite Latex 149 (47.5% T.S.) | A                                               | CC                     | PC                     | I                   | CC                     | CC                     | C                   | CC                     | PC                     | PC                  |
| 40 Styrene-60 Butadiene         | B                                               | CC                     | CC                     | C                   | CC                     | C                      | CC                  | CC                     | PC                     | PC                  |
| Pliolite Latex 160 (48.9% T.S.) | A                                               | CC                     | C                      | I                   | CC                     | PC                     | PC                  | CC                     | PC                     | PC                  |
| 33 Styrene-67 Butadiene         | B                                               | CC                     | C                      | I                   | CC                     | CC                     | C                   | CC                     | PC                     | PC                  |
| Pliolite-440 (45% T.S.)         | A                                               | CC                     | I                      | I                   | CC                     | CC                     | CC                  | CC                     | PC                     | PC                  |
| 35 Styrene-65 Butadiene         | B                                               | CC                     | PC                     | PC                  | CC                     | CC                     | C                   | CC                     | CC                     | CC                  |
| Dylex K-40 (48.9% T.S.)         | A                                               | CC                     | PC                     | PC                  | CC                     | CC                     | C                   | CC                     | CC                     | CC                  |
| 60 Styrene-40 Butadiene         | B                                               | CC                     | C                      | PC                  | CC                     | PC                     | I                   | CC                     | PC                     | PC                  |
| Celanese VX-567 (50% T.S.)      | A                                               | CC                     | C                      | PC                  | CC                     | CC                     | C                   | CC                     | PC                     | PC                  |
| Acrylate                        | B                                               | CC                     | C                      | PC                  | CC                     | PC                     | I                   | CC                     | PC                     | PC                  |
| Goodrich 450X3 (54.9% T.S.)     | A                                               | CC                     | C                      | PC                  | CC                     | PC                     | I                   | CC                     | PC                     | PC                  |
| Polyvinyl Chloride-Acrylic      | B                                               | CC                     | C                      | CC                  | CC                     | I                      | I                   | CC                     | I                      | I                   |
| Hycar-1571 (41% T.S.)           | A                                               | CC                     | C*                     | C*                  | C*                     | C*                     | I                   | CC                     | C*                     | C*                  |
| Acrylonitrile-Butadiene         | B                                               | CC                     | C                      | CC                  | CC                     | C                      | C                   | CC                     | CC                     | CC                  |
| Hycar-2671 (50.3% T.S.)         | A                                               | CC                     | C*                     | PC*                 | C*                     | C*                     | PC*                 | CC                     | C*                     | C*                  |
| Acrylate                        | B                                               | CC                     | C                      | CC                  | CC                     | C                      | C                   | CC                     | C                      | C                   |
| Rhoplex HA-8 (46% T.S.)         | A                                               | CC                     | CC                     | CC                  | CC                     | CC                     | PC                  | CC                     | PC                     | PC                  |
| Acrylate                        | B                                               | CC                     | CC                     | CC                  | CC                     | CC                     | PC                  | CC                     | PC                     | PC                  |
| Rhoplex HA-16 (46% T.S.)        | A                                               | CC                     | C                      | CC                  | CC                     | PC                     | PC                  | CC                     | CC                     | CC                  |
| Acrylate                        | B                                               | CC                     | C                      | CC                  | CC                     | PC                     | PC                  | CC                     | CC                     | CC                  |

TABLE IX—Continued

| Test Polymer               |   | Ratio of Methyol Amide of Example I to Polymer |                        |                        |                    |                        |                        |                    |                        |                        |  |
|----------------------------|---|------------------------------------------------|------------------------|------------------------|--------------------|------------------------|------------------------|--------------------|------------------------|------------------------|--|
|                            |   | 1:4                                            |                        |                        | 1:1                |                        |                        | 4:1                |                        |                        |  |
|                            |   | Imme-<br>di-<br>te                             | 8 hours on<br>standing | 24 hours<br>at 125° F. | Imme-<br>di-<br>te | 8 hours on<br>standing | 24 hours<br>at 125° F. | Imme-<br>di-<br>te | 8 hours on<br>standing | 24 hours<br>at 125° F. |  |
| Rhoplex A C-55 (55% T.S.)  | A | C                                              | PC*                    | PC*                    | C                  | C*                     | PC*                    | C                  | C                      | C                      |  |
| Acrylate                   | B | C                                              | C                      | C                      | C                  | C                      | C                      | I                  | I                      | I                      |  |
| Shawinigan 0566 (50% T.S.) | A | C                                              | C                      | C                      | C                  | PC                     | PC                     | PC                 | PC                     | PC                     |  |
| Polyvinyl Butyral          | B | C                                              | C                      | C                      | C                  | I                      | C                      | PC                 | I                      | PC                     |  |
| Poly-EM                    | A | C                                              | C                      | C                      | C                  | PC                     | PC                     | PC                 | PC                     | PC                     |  |
| Polyethylene               | B | C                                              | C                      | C                      | C                  | C                      | C                      | C                  | C                      | C                      |  |

Since many embodiments of this invention may be made and since many changes may be made in the embodiments described, the foregoing is to be interpreted as illustrative only and our invention is defined by the claims appended hereafter.

We claim:

1. A non-woven fibrous product in which the fibers are distributed in random array and bonded together by a binder wherein said binder which is cured to an insoluble condition in an uncured state comprises a water-dispersible methyol amide of an adduct formed by reaction between a maleyl compound and an ethylenically unsaturated aliphatic compound having a chain of from 10 to 24 carbon atoms containing on an average at least 2 potentially reactive carboxy groups.

2. The article of claim 1, wherein said ethylenically unsaturated compound comprises an ethylenically unsaturated fatty acid ester of a polyhydric alcohol.

3. The article of claim 2, wherein said maleyl compound comprises a compound selected from the group consisting of maleic anhydride and maleic acid.

4. The article of claim 3, wherein said said ethylenically unsaturated fatty acid ester of a polyhydric alcohol comprises an ethylenically unsaturated glyceride oil.

5. The article of claim 4, wherein said methyol amide contains on an average at least 4 potentially reactive carboxy groups.

6. The article of claim 5, wherein said binder also comprises an addition polymer of at least one monomer selected from the group consisting of ethylene, vinyl acetate, an alkyl ester of acrylic acid and an alkyl ester of methacrylic acid.

7. A non-woven fibrous product in which the fibers are distributed in random array and bonded together by a binder wherein said binder which is cured to an insoluble condition in an uncured state comprises a water-soluble product prepared by the steps of (1) reacting a compound containing a basic nitrogen atom with an adduct formed by reaction between a maleyl compound and an ester of an ethylenically unsaturated fatty acid of from 10 to 24 carbon atoms with a polyhydric alcohol having from 2 to 6 hydroxyl groups, wherein said adduct contains on an average at least 4 potentially reactive carboxy groups per molecule, and (2) reacting an aqueous solution of the reaction product of step (1) with formaldehyde.

8. The article of claim 7, wherein said maleyl compound comprises a compound selected from the group consisting of maleic anhydride and maleic acid, and said compound containing a basic nitrogen atom comprises ammonia.

9. The article of claim 8 wherein at least one-half mole

of ammonia is added in step (1) per each potentially reactive carboxy group in said adduct and at least about 0.7 mole of formaldehyde is added in step (2) per each equivalent of nitrogen containing compound bearing an NH group.

10. The article of claim 8, wherein said compound containing a basic nitrogen atom also comprises ethylene diamine.

11. The article of claim 9, wherein said ester of a polyhydric alcohol and an ethylenically unsaturated fatty acid ester comprises an ethylenically unsaturated glyceride oil.

12. The article of claim 8, wherein said binder also comprises a polymer of vinyl acetate.

13. The article of claim 8, wherein said binder also comprises a polymer of ethylene.

14. A process of making a non-woven fabric which comprises associating a mass of fibers in random array within a web, bringing into contact with said fibers an aqueous dispersion containing 1 to 60% by weight of a binder, wherein said binder comprises a water-dispersible methyol amide of an adduct formed by reaction between a maleyl compound and an ethylenically unsaturated aliphatic compound having a chain of from 10 to 24 carbon atoms containing on an average at least 2 potentially reactive carboxy groups, drying the fibrous mat containing said binder and curing the binder to an insoluble infusible condition.

15. The process of claim 14, wherein said ethylenically unsaturated compound comprises an ethylenically unsaturated fatty acid ester of a polyhydric alcohol.

16. The process of claim 15, wherein said maleyl compound comprises a compound selected from the group consisting of maleic anhydride and maleic acid.

17. The process of claim 16, wherein said ethylenically unsaturated fatty acid ester of a polyhydric alcohol comprises an ethylenically unsaturated glyceride oil.

18. The process of claim 17, wherein said methyol amide contains on an average at least 4 potentially reactive carboxy groups.

#### References Cited

#### UNITED STATES PATENTS

|    |           |         |              |           |
|----|-----------|---------|--------------|-----------|
| 60 | 2,188,885 | 1/1940  | Clockier     | 260—404 X |
|    | 2,355,265 | 8/1944  | Bock et al.  | 117—161 X |
|    | 2,637,663 | 5/1953  | Thurston     | 117—167 X |
|    | 2,833,283 | 5/1958  | Spahr et al. | 117—140 X |
|    | 2,915,418 | 12/1959 | Wolfson      | 117—140   |

65 WILLIAM D. MARTIN, Primary Examiner.

T. G. DAVIS, Assistant Examiner.

UNITED STATES PATENT OFFICE  
CERTIFICATE OF CORRECTION

Patent No. 3,345,207

October 3, 1967

George W. Cogswell et al.

It is hereby certified that error appears in the above numbered patent requiring correction and that the said Letters Patent should read as corrected below.

Column 1, line 60, for "within" read -- without --; column 2, line 19, for "longe" read -- long --; line 62, for "25" read -- 24 --; column 3, line 5, for "acid citraconic anhydride, itaconic acid itaconic" read -- acid, citraconic anhydride, itaconic acid, itaconic --; column 4, line 37, for "10% to 3%" read -- 10% to 33% --; column 5, line 63, for "ring" read -- ring) --; column 7, line 61, for "portion" read -- proportion --; column 8, line 10, for "disposition" read -- deposition --; line 11, for "instead" read -- Instead --; column 10, line 40, for "of a a methanol" read -- of a methylol --; column 12, line 20, for "webs" read -- web --; column 13, line 27, for "an", first occurrence, read -- and --; column 14, line 37, for "aduct" read -- adduct --.

Signed and sealed this 22nd day of April 1969.

(SEAL)

Attest:

EDWARD M. FLETCHER, JR.  
Attesting Officer

EDWARD J. BRENNER  
Commissioner of Patents